

F. A. HEADSON.

GEAR.

APPLICATION FILED SEPT. 18, 1913. RENEWED SEPT. 27, 1915.

1,180,495.

Patented Apr. 25, 1916.

*Fig. 1.*



*Fig. 2.*



*Witnesses:*

John E. Ryland,

Chas. H. Quell,

*Inventor:*

Frank A. Headson,

By Boles & Cromer  
Atkins.

# UNITED STATES PATENT OFFICE.

FRANK A. HEADSON, OF MILWAUKEE, WISCONSIN, ASSIGNOR TO H. W. JOHNS-  
MANVILLE COMPANY, OF MILWAUKEE, WISCONSIN, A CORPORATION OF  
NEW YORK.

## GEAR.

1,180,495.

Specification of Letters Patent. Patented Apr. 25, 1916.

Application filed September 18, 1913, Serial No. 790,513. Renewed September 27, 1915. Serial No. 52,961.

*To all whom it may concern:*

Be it known that I, FRANK A. HEADSON, a citizen of the United States, and a resident of Milwaukee, in the county of Milwaukee 5 and State of Wisconsin, have invented certain new and useful Improvements in Gears; and I do hereby declare that the following is a full, clear, and exact description thereof, reference being had to the accompanying drawings, and to the letters of reference marked thereon, which form a part of this specification.

This invention relates to compression gears and particularly to that class of gears 15 formed of a composition comprising fibrous asbestos and rubber cement or cementitious material.

The principal object of the invention is to provide a simple, economical and efficient 20 gear and more particularly to provide a gear which is practically noiseless, waterproof and oil-proof and a non-conductor of electricity.

Other and further objects of the invention 25 will appear from an examination of the accompanying drawings which are made a part hereof and from the following description and claims.

The invention consists in the features, 30 combinations of elements, and details of construction herein described and claimed.

In the accompanying drawings—Figure 1 is a view in side elevation of a gear constructed in accordance with my invention 35 and improvements, and showing a portion of a metallic end plate or housing secured thereto or forming a part thereof, the gear being shown keyed to a shaft; and Fig. 2, a central sectional view of the parts shown 40 in Fig. 1 with the shaft shown in elevation.

The gear shown in the accompanying drawings consists of a body portion *a* having teeth *b* integral with the body portion and all formed, by preference, of non-metallic material, and which body portion and teeth may be of any desired form adapted to accomplish the purposes for which the gear is intended to be used, and which non-metallic body portion or gear is adapted to 50 be mounted between metallic end plates or housing members *c* which may be of any desired, ordinary or known form and which may be secured to the non-metallic body portion *a* by means of bolts *d*, or other suitable securing means.

The non-metallic body portion of the gear thus formed is adapted to be used either with or without the metallic end plates or housing members and to be secured to a shaft *d* by means of a key *f*, or 60 other suitable securing means.

In constructing a gear in accordance with my invention, I provide a suitable quantity of material consisting of or including fibrous material and a binder of cementitious 65 material adapted to be compressed and vulcanized.

The first mentioned element consists, by preference, of fibrous asbestos, although a relatively small proportion of organic 70 fibrous material, such as hemp, jute or similar organic fibrous material may be used. The second element or binder consists, by preference, of cementitious material containing rubber and a filler 75 or body-forming material. The body-forming material of the binder may consist of or comprise zinc, whiting, a barium sulfate compound, such for example as barytes, blue lead or sulfur, or either 80 of these in combination with any one or all of the other of said elements. A very desirable form of binder comprises or consists of the following elements, in approximately the proportions mentioned: rubber 30%, 85 barytes 39%, pulp 5%, lime 2%, litharge 2%, sulfur 8%, blue lead 10%.

The material or composition of which the gear or non-metallic body of the article is to be made in accordance with my invention 90 and improvements thus consists, by preference, of or comprises the above mentioned elements in approximately the following proportions: fibrous material or asbestos, or the first element, 70%, and rubber or cementitious material forming a binder, or 95 the second element 30%.

The relative proportions of the elements above mentioned are by weight and may be varied to a considerable extent, as desired, 100 or as required by varying conditions. The composition may consist of 90% fiber and 10% binder or cementitious material, or the proportion of cementitious material including rubber may be increased to 50% of 105 the mass, the remaining 50% consisting of fibrous asbestos or fibrous material; and the relative proportions of the elements forming the binder may also be varied to a considerable extent and the binder may consist 110

substantially or wholly of rubber and barytes and sulfur, although I prefer to use the elements above mentioned in substantially the proportions above set forth.

The fibrous material may consist of or comprise remnants or fragments of asbestos cloth or fabric, such as is used in or produced incidental to or during the manufacture of packing, belts or similar articles of manufacture containing fibrous material or asbestos.

The fibrous material or asbestos, whether in the form of new or raw asbestos or in the form of remnants or fragments of asbestos or asbestos cloth or fabric, is ground or thoroughly disintegrated or reduced to a finely divided or pulp like condition in any desired, ordinary or well known manner, and is thoroughly intermixed with the binder or with the desired quantity of rubber or cementitious material comprising rubber or with what is known as rubber cement. The rubber when consisting in part of remnants of packing, belting or other articles containing rubber is immersed in or subjected to the action of benzin or gasoline which serves to cut or dissolve the rubber so as to provide a suitable rubber solution, the gasoline or benzin being allowed to evaporate. The rubber solution, whether formed of remnants of packing, belting or other articles or of new rubber or fresh cementitious material, is intermixed with the fibrous material while the rubber or rubber solution is in a liquid or semi-vulcanized or semi-cured condition. A pulp or mass of material is thus obtained which comprises rubber or cementitious material containing rubber in a liquid plastic or semi-vulcanized condition and fibrous material, preferably in the form of asbestos. The pulp or mass including fibrous material and rubber or cementitious material thus provided, is thoroughly intermixed and placed in a mold while the rubber solution is in a liquid or semi-vulcanized condition and the mass in a plastic condition and is subjected to pressure and sufficient heat to vulcanize the rubber or rubber solution, as hereinafter more particularly described, the pressure and heat being sufficient and being so applied as to reduce the mass to the desired density, size and shape. A suitable quantity of bakelite may be used in connection with the rubber and fibrous material or may be used in lieu of any desired quantity of rubber, although rubber is preferable.

The mold may be of any desired, ordinary or well known form of mold provided with suitable means for applying the required pressure and sufficient heat for vulcanizing the rubber or rubber solution or mass and it is therefore deemed unnecessary to illustrate or describe such mold herein. The mold should have side and end walls and upper and lower, relatively movable mold

plates, all adapted to form a mold chamber having the same shape and dimensions as the article or molded piece to be obtained. The chamber formed by the mold being of such dimensions that when the mold plates are separated the mold will admit between the side and end walls and top and bottom or movable and stationary plates of the mold the required quantity of pulp or compressible material for forming the desired blank or gear—the portion of the blank or body of which the gear teeth are to be formed containing, by preference, sufficient material or stock to enable gear teeth of suitable form to be cut.

The required heat is applied, by preference, by admitting steam into contact with the mold plates or with the mold plates and mold during the operation of compressing the pulp or material, although it is possible to first compress the material and then, before vulcanizing it or partially vulcanizing, to place it in a form and then subject it to heat sufficient to vulcanize the rubber or cementitious material or the mass comprising the fibrous material and cementitious material or binder. The pulp or compressible material is allowed to cool after being subjected to the required degree of heat and pressure or to the action of steam at the required temperature and for the required length of time to suitably vulcanize the material. A hydraulic pressure of 5000 pounds to the square inch, applied, by preference, while the material is in a heated condition, 100 preferably at a temperature of 300° F. and while the material is in a plastic or compressible condition, is found in practice to be sufficient to accomplish the desired result. In practice the mass is reduced by means of the pressure and during the process of vulcanizing to approximately one-fourth or even one-fifth of the original normal bulk of the mass. The pressure sufficient to maintain the mass in this highly compressed condition is maintained, by preference, during the vulcanizing and also during the cooling of the material or until the material thus compressed in a plastic condition is allowed to cool, set and harden. The body of the finished article is thus exceedingly dense, compact and strong. The temperature should be maintained, by preference at or above 250° F. and below 600° F. and such temperature and required pressure should be maintained for about thirty minutes, the pressure being continued as already suggested during the cooling of the material or for any desired period in excess of the period of time during which the vulcanizing is accomplished.

When remnants or fragments of asbestos cloth or fabric are used, such remnants or fragments may be found to contain a quantity of metal ordinarily in the form of cop-

per or brass wire or particles of copper or brass to the extent of 2%, more or less, of the mass of fibrous material. In such cases the copper or metal is finely ground or disintegrated to such an extent as to consist of exceedingly small particles which, by preference, should not exceed in size the particles of ordinary metal fillings or fine powder, such particles being embedded in the mass and surrounded by the fibrous material and binder or non-conductor.

Articles containing a very small proportion of metal thus intermixed with the non-metallic material are adapted to be used when the electrical conductivity or non-conductivity of the material is unimportant, but the non-metallic elements should be used without any metal being intermixed therewith when the article or gear is to be a non-conductor of electricity and the article or gear embodying my invention or improvements in its preferred form is by preference formed wholly of non-metallic material intermixed, molded and vulcanized in the manner above described.

A gear or article constructed or formed of the composition or material above described has the advantage of being practically noiseless in operation and of being a non-conductor of electricity. It is practically water-proof and oil-proof and will not become excessively hot or overheated as a result of frictional engagement with other parts when in operation. It will not wear away faster when overheated in any manner, by extraneous means or otherwise, than when at the ordinary atmospheric temperature and will not unduly expand or contract with variations in temperature. It is sufficiently strong to withstand all stresses and strains to which such a gear or article is of necessity subjected in use, and has great durability and strength.

I claim:

1. A gear or other article of the class described, comprising in combination, fibrous asbestos, cementitious material containing rubber, and a barium sulfate compound, all compressed together and vulcanized. 45

2. A gear of the class described, comprising in combination, fibrous asbestos, cementitious material containing rubber, barytes, and sulfur, all compressed together to a density in excess of the normal density of the mass and vulcanized. 50 55

3. A nonmetallic gear, comprising fibrous asbestos, and a binder containing rubber, barytes, and sulfur, all compressed together and condensed to less than one-fourth of the original bulk of the mass and vulcanized. 60

4. A gear body of the class described formed of a composition comprising, in combination, fibrous asbestos, cementitious material containing rubber and sulfur, and a filler having the characteristics of a finely divided solid mineral substance all intermixed in the form of a pulp and compressed into a rigid mass and vulcanized. 65

5. A gear body of the class described formed of a composition comprising, in combination, fibrous asbestos, cementitious material containing rubber and sulfur, and a filler having the characteristics of a finely divided solid mineral substance, including disintegrated metal, all intermixed in the form of a pulp and compressed into a rigid mass and vulcanized. 70 75

In testimony that I claim the foregoing as my invention I affix my signature in the presence of two witnesses, this 15th day of September, A. D. 1913. 80

FRANK A. HEADSON.

Witnesses:

W.M. T. BAIN,  
J. L. ACHTERBERG.